

## UNITED STATES PATENT OFFICE

FRANK H. DRIGGS, OF BLOOMFIELD, NEW JERSEY, ASSIGNOR TO WESTINGHOUSE LAMP COMPANY, A CORPORATION OF PENNSYLVANIA

PREPARATION OF RARE METALS BY ELECTROLYTIC DECOMPOSITION OF THEIR FUSED DOUBLE HALOGEN COMPOUNDS

No Drawing.

Application filed May 11, 1928. Serial No. 277,096.

This invention relates to the art of metallurgy and more particularly relates to the art of electro-metallurgy and comprises essentially a method of preparing rare refractory metal powders of substantial purity and freedom from deleterious impurities by electrolytically depositing the same from a fused halogen bath containing an ionizable halogen compound of the rare refractory metal, recovering the metal powder from the fusion mixture by suitable lixiviation means, thereafter compacting and sintering the metal powder in an inert environment to a coherent ductile body.

Heretofore many methods have been devised for the preparation of the so-called rare refractory metals. Most of these methods have been directed to the production of the metal by reducing compounds of the same with highly reactive metals such as sodium, magnesium, aluminum and calcium. Due to the extreme activity of the rare refractory metals in the powder state, great difficulty has been encountered in preparing them substantially free from deleterious impurities of carbon, nitrogen, oxygen, etc. Such reduction methods as have heretofore been developed have been relatively expensive to operate.

Specifically, this invention is directed to the production of the rare refractory metal uranium by the electrolytic decomposition of its ionized fused halogen salts. Heretofore it has been considered that the high chemical activity of uranium would prevent the preparation of the metal by such electrolytic methods, but I have developed a method whereby such electrolytic decomposition of uranium salts may be effected.

One of the objects of this invention is to provide a method of producing rare refractory metals by electrolytic decomposition of their fused halogen compounds.

Another object of this invention is to provide a method of preparing uranium by the electrolytic decomposition of fused uranium halogen compounds.

Another object of this invention is to provide a method whereby uranium metal may be prepared by electrolytic decomposition of

fused double halogen compounds of uranium with the alkali metals.

Another object is to provide a cheaper and more efficient method than heretofore available for the production of uranium metal powders.

Another object of this invention is to provide a means of recovering the uranium and other refractory metal powders from the fused bath and to compact and sinter the same into coherent metal bodies which may subsequently be mechanically deformed into shapes useful in the arts.

Other objects and advantages will become apparent as the process is described.

In the preparation of uranium by my process I preferably employ as an ionizable halogen compound of the metal an anhydrous double halogen compound of an alkaline metal with uranium and specifically I prefer to use the double fluoride compound of uranium with potassium, having a formula  $KUF_5$ . This salt may be prepared as set forth in copending application Serial No. 168,826, entitled Preparation of an oxide-free halide of a rare refractory metal, and assigned to the same assignee as the present invention.

The reasons why I prefer to use this particular double alkaline uranium compound in the electrolytic preparation of uranium are as follows: In the first place, I have found that in order to prepare substantially pure uranium I must use substantially pure uranium compounds in the electrolytic process and that this method of crystallizing uranium double fluorides ensures absolute purity as regards the uranium salt.

Secondly, I have found that fluoride fusions of uranium are more stable than chlorides, bromides, or iodides in the open air and do not tend to break down and form oxygen compounds by reaction with atmospheric oxygen. A third factor influencing the selection of this compound has been that oxygen reacts with uranium to form highly stable compounds which are insoluble and undecomposable in the alkaline fluoride fusion, and which are thereafter extremely difficult to re-

move from the metal powder which may be produced by the electrolysis procedure.

As a specific embodiment of my invention I prepare a fusion mixture comprised of approximately one part sodium fluoride (NaF) and two parts potassium fluoride (KF) which fluorides should preferably also have been purified and freed of contaminating impurities likely to be reduced to metal form 10 during the subsequent electrolysis procedure.

To this fusion mixture either prior to or after fusion I add the double alkaline fluoride compound of uranium, in such an amount as will completely dissolve in the fusion mixture, which will approximately be between twenty to twenty-five percent by weight of the total bulk of the fusion mixture employed. In solution in the fused fluoride bath, the double alkaline uranium compound being 15 instantly reduced to metal at the anode of the electric current, the uranium is liberated at the cathode and fluorine at the anode. The liberated uranium being very dense (18.7) and heavy, falls to the bottom of the fused 20 bath and is protected from reacting with the gases of the atmosphere by the fused fluoride fusion. From time to time frequent additions of alkali fluorides or of double alkali uranium fluoride may be made to render the 25 process a continuous one.

The current applied would depend upon the size of the bath, the spacing and the area of the electrodes, the rate at which it is desired to deposit the metal, and other factors. In 30 the practice of my invention I have found that a current density at the cathode of approximately .27 amperes per  $\text{cm}^2$  is nearly the correct current density. This may vary, however, depending upon the existing conditions 35 of production.

The anode current density should not be too high and I have found that .90 amperes per  $\text{cm}^2$  is approximately right to prevent the development of the so-called "anode effect" or polarizing at the anode which occurs 40 when the amount of fluorine liberated is sufficient to coat or insulate the anode from the fused bath.

The materials employed in the construction 45 of a suitable electrolytic chamber to conduct the electrolysis may be of any material which will resist the corrosive action of the fluoride fusion, namely carbon, graphite, nickel and some of the cast corrosive resistant alloys 50 such as nichrome, hardite, etc.

The electrodes may be of carbon, if desired, or of any material resistant to the corrosive action of the flux or fluorine gas liberated.

The temperature of the fused bath will 55 vary with the amount of anode effect developed and will range in the neighborhood of 700° C. to 800° C. While I have specified as a fusion mixture an alkaline fluoride fusion comprised of one part sodium fluoride (NaF) to two parts potassium fluoride (KF), it is to

be understood that such a fluoride fusion may vary within wide limits and still fall within the scope of this invention.

I may use, for instance, any other combination of the two alkaline fluorides mentioned or I may add to the bath other fluoride compounds, such as ammonium fluoride, to further "thin" the bath, or I may add thereto a proportion of any of the alkaline earth fluorides. For the reason, however,

that I must subsequently recover from the fusion the metal powder substantially free from deleterious impurities I prefer to employ in the practice of my invention those fluorides which in addition to fulfilling the other requirements of my process are capable of subsequently being removed by solution in water.

At the conclusion of the electrolysis the liberated metal powder may be recovered from the fusion in the following manner.

The fused bath is allowed to cool to room temperature in the electrolytic chamber, thereafter it may be removed and crushed to convenient small sizes. The crushed fusion mixture is then washed free of soluble fluorides by any suitable lixiviation procedure, provided means are provided for preventing the introduction of impurities such as might be caused by the formation of insoluble fluorides. I therefore prefer to conduct such lixiviation in wooden or rubber lined vessels and use very pure distilled water. After thoroughly washing free of soluble fluorides the insoluble residues may be treated with dilute nitric or acetic acids (approximately 1 part acid to 4 parts water) to dissolve out acid soluble impurities. Such acid washes should preferably be made in the cold, following which the metal powder is put through any well known minerals separation procedure to remove accompanying insoluble impurities, such as carbon, oxides, etc. Thereafter the metal powder is washed free of water by an alcohol wash followed by an ether wash, after which it is thoroughly dried in vacuo.

I have found that frequently such metal powders of uranium, prepared by my process, are pyrophoric and will spontaneously ignite and burn when exposed to the atmosphere. I have found, however, that by suitable regulation of the current density at the cathode during deposition of the metal powder to substantially increase the crystalline size thereof, such pyrophoric tendencies are mitigated, and the metal powders may subsequently be compacted, sintered and consolidated to coherent metal.

The method I may employ in the sintering and consolidation process is similar to that disclosed in copending application Serial No. 684,908, Marden et al, entitled Sintering and fusing uranium into a coherent body and which copending application is as-

signed to the same assignee as the present invention.

The process in brief, contemplates sintering and fusing (if necessary) substantially pure metal powders by initially substantially effecting degasification of the same at temperatures below the sintering temperature of the metal powder by slowly heating the powders in a high vacuo, removing the liberated adsorbed or absorbed gases as fast as they are liberated, and thereafter raising the temperature to the sintering (or fusing) temperature (if desired). In the copending application the heating has been specified as being by "inductive" heating, but, of course, any other method of heating may be applied.

Having outlined in the broadest aspect the nature of my invention and specifically directed the same to the production of uranium, it is apparent that there may be many variations of the same whereby essentially the same result may be obtained, but such variations are anticipated as may fall within the scope of my claims.

Other refractory metals may be prepared in a similar manner through the practice of my invention, such as tantalum, columbium, chromium, zirconium, thorium and the like, but those that may be so prepared are considered to fall within the scope of the term "rare refractory metals".

What is claimed is:

1. The process of preparing uranium comprising electrolytically decomposing a double halogen compound of uranium in solution in a fused bath comprised of alkali halogen compounds.

2. The process of preparing uranium comprising electrolytically decomposing a double fluoride compound of uranium in solution in a fused bath comprised of alkali metal fluorides.

3. The process of preparing uranium comprising electrolytically decomposing the double potassium uranium fluoride ( $K_2UF_6$ ) in solution in a fused bath comprised of potassium and sodium fluorides.

4. The process of preparing uranium comprised in electrolytically decomposing a fused bath composed of potassium fluoride (2 parts) sodium fluoride (1 part) potassium and uranium double fluoride up to 25 percent of the total (by weight).

In testimony whereof, I have hereunto subscribed my name this 9th day of May, 1928.

FRANK H. DRIGGS.